

## UNITED STATES PATENT OFFICE

2,080,050

SENSITIZATION OF PHOTOGRAPHIC  
EMULSIONS

John David Kendall, Ilford, England, assignor to  
Ilford Limited, Ilford, England, a British company

No Drawing. Original application April 27, 1936,  
Serial No. 76,703. Divided and this application  
September 9, 1936, Serial No. 99,965. In Great  
Britain August 3, 1934

7 Claims. (Cl. 95-7)

This application corresponds to the applications of John David Kendall, Serial No. 22,727/34, filed 3rd August, 1934 and divisional application Serial No. 6,314/36, dated 3rd August, 5 1934, which were both filed in Great Britain, and is a divisional of United States application Serial No. 76,703, filed 27th April, 1936.

This invention relates to the sensitization of photographic silver halide emulsions by incorporating in the emulsion a dye or dyes which have the property of extending the range of spectral sensitivity of the emulsion.

It is well known that the cyanine dyes, that is dyes comprising two heterocyclic nitrogen nuclei joined by a methine or polymethine chain, modify the spectral sensitivity of silver halide emulsions.

In the specification of my co-pending application No. 76,703 filed 27th April, 1936 (from which this application is divided) I have described the preparation of dyes having a structure similar to that of the cyanine dyes but containing one or two nitrogen atoms in the linking chain between the two heterocyclic nuclei. 20 I have found that when such dyes are alkyl salts, and so contain a quinquevalent nitrogen atom linked to a trivalent nitrogen atom by a completely conjugate chain, they have the property of extending the spectral sensitivity of silver halide emulsions.

In a paper in J. C. S. volume 125, (1924) page 1348, Dr. Hamer describes the preparation of 1:1'-dimethyl-2:2'-azocyanine iodide and states that a solution of this compound is pale yellow 25 with a blue fluorescence and is unlike the cyanines in that it is not decolorized by acids whilst it has no action on a photographic plate. I have found that 1:1'-dimethyl-2:2'-azocyanine iodide is a powerful sensitizer for silver halide emulsions, particularly for silver chloride emulsions and it extends the sensitivity of a silver chloride emulsion to  $\lambda$  4600 Å. with sharp maxima at 30 about  $\lambda$  4150 Å. and  $\lambda$  4400 Å. This compound is one of the class of compounds which I have now found to have sensitizing properties and I include its use as a sensitizer in the appended claims.

According to my invention a method of extending the spectral sensitivity of photographic silver halide emulsions (particularly silver chloride emulsions) comprises treating the emulsion with a compound containing two heterocyclic nitrogen nuclei (one of which contains a trivalent and the other a quinquevalent nitrogen atom) which are linked in the  $\alpha$  or  $\gamma$  positions

to the nitrogen atoms by a linkage selected from the group consisting of  $-\text{N}=\text{}$ ,  $-\text{CH}=\text{CH}-\text{N}=\text{}$ ,  $-\text{N}=\text{CH}-\text{N}=\text{}$  or  $-\text{N}=\text{CX}-\text{N}=\text{}$  (X representing a hydrocarbon group).

The invention also includes a photographic silver halide emulsion containing one of the above-mentioned compounds.

In carrying out my invention I find that it is preferable to use the compounds containing the chain  $-\text{CH}=\text{CH}-\text{N}=\text{}$  when it is desired to 10 extend the spectral sensitivity of a silver bromide or iodobromide emulsion.

The class of compounds which may be employed in accordance with the invention is illustrated by the following typical examples:—



20



25



30



35

40

It will be understood that in the compounds which may be employed as sensitizers in accordance with my invention, the nuclei attached to the ends of the chains may be any of the heterocyclic nuclei usually occupying similar positions in the analogous cyanine compounds, for example pyridines, quinolines, naphthaquinolines or their homologues, thiazoles, oxazoles, selenazoles, diazoles (such as pyrimidines, thiadiazoles and other heterocyclic ring compounds containing two nitrogen atoms in the same ring, as described in British Patent No. 425,609) and their homologues in the benzene, naphthalene and homologous series, and the nuclei attached to 45 50 55

the ends of the chain may be different from one another, but in the case of the compounds having the linkage  $-\text{N}=\text{CH}-\text{N}=$  the nuclei will normally be the same.

5 The sensitizing action of the dyes which may be used in accordance with the present invention is illustrated by the following typical examples of compounds which may be employed. These examples are merely given as an illustration of the type of compound which may be employed.

(1) 2:1'-dimethyl-1:2'-thioquinocyazine iodide (prepared by fusing together 1-amino-benzthiazole, 2-methylmercapto-quinoline and methyl-p-toluene sulphonate, extracting with pyridine and pouring into aqueous solution of potassium iodide) extends the spectral sensitivity of a silver chloride emulsion to about  $\lambda$  4700 Å. with a maximum at about  $\lambda$  4350 Å.

20 (2) 2:2'-dimethyl-thio-oxacyazine iodide (prepared in a manner similar to that of (1) except that 1-methylmercapto-benzoxazole is employed) extends the sensitivity of a silver chloride emulsion to about  $\lambda$  4100 Å. with a maximum at about 25  $\lambda$  3780 Å.

(3) 2:2'-dimethyloxacyazine iodide (prepared by fusing together 1-amino-benzoxazole methyl-p-toluene sulphonate and 1-methylmercapto-benzoxazole methyl-p-toluene sulphonate, and pouring a solution into an aqueous solution of potassium iodide) is a weak sensitizer for silver chloride emulsions.

(4) 2:2'-dimethylthiocyazine-p-toluene sulphonate (prepared by fusing together 1-amino-benzthiazole, 1-methylmercapto-benzthiazole and methyl-p-toluene sulphonate) extends the sensitivity of silver chloride emulsions to about  $\lambda$  4200 Å. with a maximum at about  $\lambda$  3980 Å.

(5) 2:2'-dimethylthiocydiazine iodide (prepared by fusing together 1:1'-dibenzthiazolyl formamidine and methyl-p-toluene sulphonate, extracting with pyridine and pouring into an aqueous solution of potassium iodide) extends the sensitivity of silver chloride emulsions to about 45  $\lambda$  4200 Å. with a maximum at about  $\lambda$  4000 Å.

(6) 2:2'-dimethyl-5:6-benzthiocyazine iodide (prepared by fusing together 1-amino- $\alpha$ -naphtha thiazole, 1-methylmercapto benzthiazole and methyl-p-toluene sulphonate, extracting with pyridine and pouring into an aqueous solution of potassium iodide) extends the sensitivity of silver chloride emulsions to about  $\lambda$  4300 Å. with a maximum at about  $\lambda$  4150 Å.

(7) 2:1'-dimethyl-1:4'-thioquino-cyazine iodide (prepared by fusing together 1-ethyl-quinoline-4-thione, 1-amino-benzthiazole and methyl-p-toluene sulphonate, extracting with pyridine and pouring into an aqueous solution of potassium iodide) extends the sensitivity of silver chloride emulsions to about  $\lambda$  4800 Å. with a maximum at about  $\lambda$  4500 Å.

(8) 1:1'-dimethyl-2:2'-quinocyazine iodide is a powerful sensitizer for silver chloride emulsions, extending the sensitivity to about  $\lambda$  4600 Å. with sharp maxima at about  $\lambda$  4150 Å. and  $\lambda$  4400 Å.

(9) 1:1'-dimethyl-2:4'-quinocyazine iodide (prepared by condensing 2-methylmercapto-quinoline methyl-p-toluene sulphonate with 4-amino-quinoline methiodide in the presence of sodium ethylate) extends the sensitivity of a silver chloride emulsion to about  $\lambda$  4800 Å. with sharp maxima at about  $\lambda$  4250 Å. and  $\lambda$  4550 Å.

(10) 1:1'-dimethyl-4:4'-quinocyazine iodide 75 (prepared by condensing  $\text{N}$ -methyl-quinoline-4-

thione methyl-p-toluene sulphonate with 4-aminoquinoline methiodide in the presence of sodium ethylate) extends the sensitivity of a silver chloride emulsion to about  $\lambda$  5000 Å. with a sharp maximum at about  $\lambda$  4550 Å. and a less marked maximum at about  $\lambda$  4825 Å.

(11) 2:1'-dimethyl-1:2'-thiopyridoquiazine iodide increases the normal sensitivity of a silver chloride emulsion and extends the range to about  $\lambda$  4200 Å. with a maximum at about  $\lambda$  3925 Å. 10

(12) 1:1'-dimethyl-2:2'-pyridoquiazine iodide increases the normal sensitivity of silver chloride emulsions and extends the range to about  $\lambda$  4300 Å. with an indeterminate maximum at 15 about  $\lambda$  4150 Å.

(13) 2:2'-dimethyl-4':5'-methylenedioxy-thio-selenocyazine-p-toluene sulphonate extends the sensitivity of silver chloride emulsions to about  $\lambda$  4500 Å. with indeterminate maxima at about 20  $\lambda$  4150 Å. and  $\lambda$  4300 Å.

(14) 2:3'-dimethyl-2'-methylthiol-1:4'-thiopyrimidocyazine iodide increases the normal sensitivity of silver chloride emulsions and extends the range to about  $\lambda$  4200 Å. 25

(15) 2:3'-dimethyl-1:4'-thioquinazolinocyazine iodide extends the sensitivity of silver chloride emulsions to about  $\lambda$  4600 Å. with indeterminate maxima at about  $\lambda$  4000 Å. and  $\lambda$  4400 Å.

(16) 2-methyl-2'-ethylcarbothiocyazine iodide 30 (prepared by condensation of 1-aminobenzthiazole ethobromide and 1- $\omega$ -acetanilidovinyl benzthiazole methiodide in pyridine solution) extends the sensitivity of silver chloride emulsions to about  $\lambda$  5200 Å. with maxima at about  $\lambda$  4600 Å. 35 and  $\lambda$  4900 Å.

(17) 1:3:3:1'-tetramethyl-2:4'-indocarboquino-cyazine iodide (prepared by condensation of 4-amino quinoline methiodide and 1:3:3-trimethyl-2- $\omega$ -acetanilidovinyl indolene iodide in the presence of sodium ethylate) extends the sensitivity 40 of a silver bromide emulsion to about  $\lambda$  6200 Å. with a maximum at about  $\lambda$  5750 Å.

(18) 1:3:3-trimethyl-1'-ethyl-1:2'-indocarboquino-cyazine iodide (prepared in a manner similar to that of (17) except that 2-amino-quinoline ethiodide is employed) extends the sensitivity of a silver chloride emulsion to about  $\lambda$  5200 Å. with maxima at about  $\lambda$  4950 Å. and  $\lambda$  4550 Å. 45

(19) 2:2'-dimethylthiocyazine iodide (prepared by fusing together 1-amino-benzthiazole, 1-methylmercapto-benzthiazole and methyl-p-toluene sulphonate, extracting with pyridine and pouring into an aqueous solution of potassium iodide) extends the sensitivity of a silver chloride emulsion to about  $\lambda$  4100 Å. with a maximum at about  $\lambda$  3950 Å. 55

The nomenclature which I have adopted in this specification and claims may be explained 60 as follows:

Cyazine—an alkyl salt containing two heterocyclic rings containing a ring nitrogen atom linked by a single nitrogen atom ( $-\text{N}=\text{}$ ) in the alpha or gamma position after the manner shown 65 in the above formulae.

Cyadiazine—an alkyl salt containing two heterocyclic rings containing a ring nitrogen atom linked by the chain  $-\text{N}=\text{CH}-\text{N}=$  in the alpha or gamma position after the manner shown in 70 the above formulae.

Carbocyezine—an alkyl salt containing two heterocyclic rings containing a ring nitrogen atom linked by the chain  $-\text{CH}=\text{CH}-\text{N}=$  in the alpha or gamma position after the manner shown in 75

the above formulae; when the two heterocyclic nuclei are different the term indicating the nucleus attached to the  $-\text{CH}=\text{CH}-$  group of the chain precedes the term "carbo", whilst that for the nucleus attached to the nitrogen atom precedes the term "cyazine".

I claim:

1. A photographic silver chloride emulsion in which is incorporated as a sensitizer a salt of the class consisting of cyazine, cyadiazine and carbocyazine.

2. A photographic silver chloride emulsion in which is incorporated as a sensitizer a cyazine salt.

3. A photographic silver chloride emulsion in

which is incorporated as a sensitizer a carbocyazine salt.

4. A photographic silver chloride emulsion in which is incorporated as a sensitizer 2:1'-dimethyl-1:2'-thioquinocyazine iodide.

5. A photographic silver chloride emulsion in which is incorporated as a sensitizer 1:1'-dimethyl-2:2'-quinocyazine iodide.

6. A photographic silver chloride emulsion in which is incorporated as a sensitizer 1:3:3-trimethyl-1'-ethyl-1:2'-indocarboquinocyazine iodide.

7. A photographic silver chloride emulsion in which is incorporated as a sensitizer a quinocyazine salt.

5

10

15

JOHN DAVID KENDALL.